

## UNITED STATES PATENT OFFICE.

LOUIS DU PLESSIS CLEMENT, OF DOVER, DELAWARE, ASSIGNOR TO KENT COUNTY OIL CORPORATION, OF LEIPSIC, DELAWARE, A CORPORATION OF DELAWARE.

## COMPOUNDED LIQUID FUEL AND METHOD OF PRODUCING THE SAME.

No Drawing.

Application filed May 24, 1921. Serial No. 472,275.

*To all whom it may concern:*

Be it known that I, LOUIS DU PLESSIS CLEMENT, a citizen of the Kingdom of Denmark, residing at Dover, in the county of Kent and State of Delaware, have invented certain new and useful Improvements in Compounded Liquid Fuel and Methods of Producing the Same, of which the following is a specification.

10 My invention relates to liquid fuel, such as is suitable for use as a fuel for internal combustion engines such, for example, as those which are employed as motors for aeroplanes, automobiles, motor boats, and 15 other motor propelled vehicles, and my invention further relates to the process or method of compounding and producing such liquid fuel.

The object of my invention is to produce 20 a liquid fuel or compounded liquid fuel, which, when stored or transported, is relatively safe; which, in the open air, evaporates relatively slowly; which, when used as a fuel in an internal combustion engine, is more efficient and powerful than gasoline or similar fuels; which is not acid in its reaction and therefore does not have the corrosive action of many fuels on the motor or engine, and which is not liable to overheat the engine or 30 motor as do many fuels now commonly used in such motors.

Further objects of my invention will appear in the specification and claims below.

My invention and improved fuel or compounded liquid fuel is a substantially colorless liquid which, when stored in ordinary liquid fuel containers, evaporates much more slowly than gasoline, which does not readily flash or explode at atmospheric pressure, and 40 has a flashing point substantially  $35^{\circ}$  Fahr. below that which a mere untreated mechanical mixture of toluol and kerosene would have.

The ingredients which I preferably employ in preparing my new and improved fuel or compounded liquid gas and the preferred proportions thereof, by volume, and in quantities sufficient to make about 100 gallons of finished product, are as follows: 50 Toluol, 60 gallons; kerosene, 30 gallons; water, 5 gallons and upward; aluminum sulphate,  $\frac{1}{2}$  pound; bicarbonate of soda,  $\frac{1}{2}$  pound; sulphuric acid, 4 fluid ounces; bichromate of potassium, up to about 4

ounces; liquid naphtha, 21 quarts and upward.

The naphtha above indicated, and which I prefer to use in making my compounded liquid gas, is that having the highest flash test. Instead of aluminum sulphate, I may substitute a substantially equal quantity of alum ammonium.

The quality or grade of toluol which I employ is any commercial grade of toluol. I may use any of the toluols from pure toluol (toluene) down to toluol which contains a considerable amount of the next higher coal tar distillate (benzol). As a matter of fact, unless the process of distillation is carried out with great care, commercial toluol usually contains a considerable quantity of benzol, and frequently up to 2% of the next heavier distillate (xylol). I may use in my process, and with highly satisfactory results, a toluol which contains up to 50% of benzol.

The amount of water which is placed in the tank may also vary. It may be repeatedly used, but should be replaced when it contains too many of the impurities removed from the toluol and kerosene during the process. A high grade naphtha should be employed, preferably commercially pure.

My improved fuel, or compounded liquid fuel, may be produced or compounded in many different ways and in any suitable container, but I prefer to prepare the same in a steel tank having an outlet at the bottom, preferably controlled by a hand-operated valve and through which any sediment or precipitate may be drawn off from time to time, as may be found necessary or desirable. I also preferably provide the said tank with an outlet, also valve-controlled, through which the clear liquid above the precipitate or sediment, may be siphoned, decanted, or otherwise drawn off from the tank after the precipitate or sediment has settled to the bottom thereof and the liquid above the deposit has become clear. The tank may be a closed one, or one arranged to be tightly closed so that unnecessary evaporation may be prevented, and the ingredients are preferably supplied to, or put into the tank, through a relatively large opening at the top thereof capable of being tightly closed after the introduction of the ingredients into the tank. Such an inlet might be provided by a hand-hole having a

cover adapted to be tightly clamped over said hand-hole. A safety valve may be, and preferably is, in communication with the top of the tank or chamber.

5 To produce my improved compounded liquid fuel, I may substantially simultaneously introduce into the tank, through the hand-hole or other inlet at the top thereof, the toluol, kerosene, water and aluminum sulphate in substantially the proportions, by volume, above indicated. After a short time (a few minutes), the aluminum sulphate will disappear, the same having been dissolved into the water. It may well 10 here be stated that the toluol and kerosene and water, when first introduced into the tank, do not unite or combine well, at this stage of the process. They tend to separate from each other and to form superposed 15 layers in the tank, the kerosene floating on the water, and the toluol on the kerosene.

I may then substantially simultaneously 20 introduce into the tank from different containers and mix with the ingredients already contained therein, the bicarbonate of soda and sulphuric acid in substantially the proportions above set forth. The hand-hole or other inlet may be then quickly closed. The introduction of the sulphuric 25 acid and bicarbonate of soda immediately sets up a chemical agitation or ebullition of the entire contents of the tank and the aluminum sulphate will be repeatedly forced through the toluol, kerosene and 30 water, with the result that the toluol and kerosene becomes thoroughly cleansed of foreign matters and impurities, such as metallic substances or compounds, fats, heavy oils, paraffine and coloring matter. 35 The action of the aluminum sulphate appears also to be one of bringing the toluol and kerosene closely together and to form of them a unitary homogeneous substance or liquid. The tendency of the two substances, 40 toluol and kerosene, to separate out from 45 each other, particularly upon changes in atmosphere, substantially and practically disappears after this treatment, and the toluol and kerosene act no longer like mere mixture of liquids having little or no affinity for 50 each other, but they remain mixed or united together in permanent stable fluid form.

After the ebullition and chemical agitation caused by the introduction of the bicarbonate of soda and sulphuric acid has ceased, I then add the bichromate of potassium and the naphtha. The bichromate of potassium 55 appears to unite with the impurities and foreign matters above referred to, imparting to them a high yellow color and precipitating them out from the solution. The impurities, 60 therefore, which have thus been washed out of the various ingredients by the action of the aluminum sulphate and the bicarbonate 65 of soda and sulphuric acid, rapidly settle on

the bottom of the tank, leaving above the sediment or precipitate, a clear colorless liquid. This settling of impurities or solid matter requires but a relatively short time, such, for example, as from 5 to 10 minutes. 70

The liquid naphtha which is introduced at substantially the same time as the bichromate of potassium above referred to, unites or mixes with and forms a permanent part of the clear liquid. Its effect is to raise and determine or fix the volatilization point of the product. While I have here indicated 44 gallons of the naphtha as being the preferred amount to use in the treatment of 100 gallons of the mixture, 80 this amount may be suitably and substantially varied to bring the volatilization point of the resulting compounded liquid fuel high or low as desired, dependent upon the particular use to which the fuel is to be 85 put.

After the precipitate or sediment has completely settled on the bottom of the tank, the clear liquid, which is my compounded liquid fuel, may then be decanted, siphoned, pumped, or otherwise drawn off from and out of the tank in any desired manner, so long as the accumulated sediment or precipitate at the bottom of the tank is not disturbed. 90

The resulting liquid or compounded liquid fuel so drawn off from the tank, may be stored in any suitable container, preferably such as are used for containing gasoline, and may be shipped to and stored at any desired place. It will be found to have a flashing point as determined by a Bureau of Standards flash tester, of about 196° Fahrenheit or from 30° to 40° Fahr. below that which a mere untreated mixture of toluol and kerosene would have depending however, somewhat upon the amount of naphtha introduced therein. It is clear and substantially colorless. It remains stable and in its original condition, substantially unaffected by ordinary atmospheric changes. It is much safer than gasoline, because it does not readily flash at ordinary atmospheric pressures. It does not have an acid reaction. 100

While I have above described the preferred way of producing my compounded liquid gas, it is to be understood that the ingredients and the proportions thereof may be varied within reasonable limits, and that the order of the steps may also be varied, without departing from the spirit and scope of my invention. 110

Having thus described my invention, what I claim and desire to protect by Letters Patent of the United States is:

1. A liquid fuel for internal combustion engines and the like comprising a clear, colorless, homogeneous, stable liquid having a flashing point of substantially 196° Fahr. 130

and comprising toluol, kerosene and naphtha thoroughly agitated in an aqueous solution of aluminum sulphate, the toluol content being substantially twice that of the kerosene content.

2. A method of making compounded liquid fuel which consists in subjecting a mechanical mixture of toluol and kerosene in proportions of two of toluol to one of kerosene, to agitation caused by chemical reaction in an aqueous solution of aluminum sulphate and adding thereto a relatively small quantity of bichromate of potassium to precipitate the impurities therefrom, and naphtha thereto.

3. A method of making compounded liquid fuel for internal combustion engines which consists in cleansing by agitation caused by chemical reaction, a mechanical mixture of toluol and kerosene in a solution of aluminum sulphate, adding a relatively small quantity of bichromate of potassium to assist in precipitating the impurities therefrom, and naphtha thereto.

4. The method of making compounded liquid fuel, which consists in mixing and chemically agitating together, toluol, kerosene, water and aluminum sulphate, adding bichromate of potassium thereto to cause

the solid matters therein to settle adding naphtha to control and determine the point of volatilization of the resulting composition, and then decanting the clear liquid.

5. The method of making a compounded liquid fuel which consists in mixing the following ingredients in substantially the following manner and in substantially the following proportions; toluol (60 gallons), kerosene (30 gallons), water (5 gallons and upward), aluminum sulphate ( $\frac{1}{2}$  pound); adding thereto bicarbonate of soda ( $\frac{1}{2}$  pound), and sulphuric acid (4 fluid ounces); after the resulting ebullition has ceased, adding bichromate of potassium (up to about 4 ounces), and fixing the flashing point of the resulting clear liquid by adding naphtha thereto.

6. A liquid fuel for internal combustion engines produced by treating a mixture of toluol and kerosene with aqueous solutions of aluminum sulphate, bicarbonate of soda, and bichromate of potassium, and with sulphuric acid, whereby the reaction of said sulphuric acid on said bicarbonate of soda produces an ebullition throughout the in-

gredients which intimately mixes said ingredients, removes and precipitates the impurities from the toluol and kerosene and unites the toluol and kerosene into a clear, colorless, stable, homogeneous liquid.

7. A liquid fuel for internal combustion engines produced by treating a mixture of toluol and kerosene with aqueous solutions of aluminum sulphate, bicarbonate of soda, and bichromate of potassium, and with sulphuric acid, whereby the reaction of said sulphuric acid on said bicarbonate of soda produces an ebullition throughout the ingredients which intimately mixes said ingredients, removes and precipitates the impurities from the toluol and kerosene and unites the toluol and kerosene into a clear, colorless, stable, homogeneous liquid, and adding naphtha thereto.

8. A liquid fuel for internal combustion engines and the like produced by mixing toluol and kerosene in an aqueous solution of aluminum sulphate, agitating the mixture by chemical reaction by adding sulphuric acid and bicarbonate of soda thereto, precipitating impurities out of said toluol and kerosene by adding bichromate of potassium, and drawing off the clear liquid above the aqueous solution.

9. A liquid fuel for internal combustion engines produced by mixing toluol and kerosene in an aqueous solution of aluminum sulphate, agitating by chemical reaction the entire mixture by adding sulphuric acid and bicarbonate of soda thereto, precipitating impurities out of said toluol and kerosene by adding bichromate of potassium, drawing off the clear liquid above the aqueous solution, and adding naphtha thereto.

10. A liquid fuel for internal combustion engines and the like produced by mixing toluol, kerosene and water, adding thereto aluminum sulphate, bicarbonate of soda, sulphuric acid, bichromate of potassium and naphtha, whereby the reaction of the sulphuric acid on the bicarbonate of soda causes an ebullition throughout the mixture, and when the ebullition is ceased, the impurities settle in the water at the bottom of the mixture, and drawing off the clear, colorless, homogeneous, stable liquid above said water.

In witness whereof, I have hereunto set my hand this 23rd day of May, 1921.

LOUIS DU PLESSIS CLEMENT.